

# UNITED STATES PATENT OFFICE.

FREDERIC LEWIS NATHAN AND WILLIAM RINTOUL, OF STEVENSTON, AND FRANK BAKER, DECEASED, LATE OF STEVENSTON, SCOTLAND, BY HENRY BAKER ADMINISTRATOR, OF ETON, WINDSOR, ENGLAND, ASSIGNEES TO NOBEL'S EXPLOSIVES COMPANY, LIMITED, OF GLASGOW, SCOTLAND.

## PROCESS FOR PREPARING GELATINIZED PROPELLENT EXPLOSIVES.

1,302,202.

Specification of Letters Patent.

Patented Apr. 29, 1919.

No Drawing.

Application filed February 26, 1914. Serial No. 821,335.

*To all whom it may concern:*

Be it known that we, Colonel Sir FREDERIC LEWIS NATHAN and WILLIAM RINTOUL, both subjects of the King of Great Britain and Ireland, and residing at Ardeer, Stevenston, Ayrshire, Scotland, and FRANK BAKER, deceased, late of Ardeer, Stevenston, Ayrshire, Scotland, have invented a certain new and useful Improved Process for Preparing Gelatinized Propellant Explosives, of which the following is a specification.

Present day smokeless powders are generally prepared by gelatinizing nitrocellulose, either when used alone or with nitroglycerin, by a volatile solvent but this entails certain disadvantages, the drying process for removing the solvent being lengthy and, what is worse, besides tending owing to the heating to affect the stability, is incomplete, so that during storage an after-drying and slow production of irregularities in the material can occur.

In the course of investigations upon the stabilizing of nitric-ester-containing explosives we found that certain partially substituted ureas in which an aromatic radical occurs (see United States application No. 771620, Patent No. 1,090,641 granted March 17, 1914,) are particularly adapted for use for stabilization but we have further found that among these bodies some are also effective gelatinizers for mixtures of nitroglycerin and nitrocelluloses.

According to the present invention therefore we utilize one or more such substances to produce a gelatinized propellant explosive from these nitric esters, the gelatinizer remaining in the final product and acting as stabilizer.

The following is a list of some of the substances referred to which possess this double property namely:

Methyl phenyl urea,  $C_8H_{10}ON_2$ ;

Ethyl phenyl urea,  $C_9H_{12}ON_2$ ;

Methyl diphenyl urea,  $C_{14}H_{14}ON_2$ .

Moreover homologues and certain derivatives of these substances possess like properties. Thus the substitution of a methyl for an ethyl group or of a hydrogen atom in a phenyl group by the grouping  $-O.CH_3$  or  $-O.C_2H_5$  in one of the above compounds but little affects their gelatinizing and stabilizing power.

In carrying the invention out in one way 7.5 parts by weight of the selected gelatinizing and stabilizing agent are dissolved in 40 parts of nitroglycerin and this solution then incorporated by the wet incorporation method of Lundholm English Patent No. 10376 of 1889 with 52.5 parts of soluble nitrocellulose of 12.6% nitrogen content which has been prepared by nitrating cotton waste at the ordinary temperature, and purified by boiling with water.

The pasty admixture so obtained is freed as far as possible from water by pressing and rolling between rollers heated to from 40° to 50° C. after which it is again rolled at a temperature of from 50° to 70° C. and a gelatinized sheet of the desired thickness obtained which is either cut into strips or flakes or extruded from a press, the pressure required in the latter (usually some hundreds of atmospheres) falling with rise in the temperature adopted which may conveniently be between 50 and 70° C.

The bodies considered vary in their gelatinizing effect and the solution of the material to be used in any particular case also depends largely upon the nature of the nitrocellulose to be treated, a powerful gelatinizer like methyl phenyl urea being more suitable for gun cotton or insoluble nitrocellulose than weak gelatinizers which may be quite satisfactory for nitrocellulose of the kind employed in making celluloid. Again the greater the proportion of nitrocellulose in the mixture the more effective the gelatinizer, which has both to colloid the fibrous nitrocellulose and to increase the plasticity of the final product, should be.

As certain of the bodies are better gelatinizers than stabilizers or vice versa it may be convenient to use mixtures thereof, the poorer gelatinizing power of the one being compensated by the better gelatinizing power of the other and vice versa as regards their stabilizing effects.

The amount of the gelatinizing and stabilizing agent or agents used will vary but generally be between 5 and 12% of the whole mixture.

The physical properties of the agent or agents used will affect the above method of introduction into the mixture for while liquid bodies are easily dissolved in the ni-

troglycerin, solids require to be finely ground and thoroughly agitated with the nitroglycerin or to be melted, if of low fusing point, and so added to the nitroglycerin. By admixture the melting point may be reduced, a mixture of some of these bodies which separately are solid being more or less liquid at temperatures but little above normal. Where the substance or substances used is or are soluble in water and the wet incorporation method is used, the suspension should be effected in a solution of the substance or substances of such strength that having regard to the mixture used the right final composition results. Thus for a mixture of 35% nitroglycerin, 55% of soluble nitrocellulose (12.6% nitrogen) and 10% gelatinizer the suspension should be effected in a 3.86% solution of methyl phenyl urea where the latter is used as gelatinizing and stabilizing agent.

Having now described our invention, what we claim as new and desire to secure by Letters Patent is:—

25 1. The process for producing a gelatinized and stabilized propellant explosive which comprises mixing together nitroglycerin, nitrocellulose and a urea derivative containing in the amido groups at least one unsubstituted hydrogen atom, and at least one aromatic radical capable both of gelatinizing nitrocellulose and of stabilizing nitric esters, and a second body also possessing both these properties one of the latter two 30 bodies possessing the first mentioned property to a smaller extent and the second mentioned property to a larger extent than the second mentioned body, and then gelatinizing the mixture.

40 2. The process for producing a gelatinized and stabilized propellant explosive which comprises mixing together nitroglycerin, nitrocellulose and methyl phenyl urea capable both of gelatinizing nitrocellulose and of stabilizing nitric esters, and a second body also possessing both these properties one of the latter two bodies possessing

the first mentioned property to a smaller extent and the second mentioned property to a larger extent than the second mentioned body, and then gelatinizing the mixture.

3. A gelatinized and stabilized propellant explosive comprising nitroglycerin, nitrocellulose and a urea derivative containing 55 in the amido groups at least one unsubstituted hydrogen atom, and at least one aromatic radical capable both of gelatinizing nitrocellulose and of stabilizing nitric esters, and another stabilizing and gelatinizing 60 compound also possessing both these properties one of the two gelatinizing and stabilizing compounds possessing the first mentioned property to a smaller extent and the second mentioned property to a larger extent than the other gelatinizing and stabilizing compound.

4. A gelatinized and stabilized propellant explosive comprising nitroglycerin, nitrocellulose and methyl phenyl urea capable 70 both of gelatinizing nitrocellulose and of stabilizing nitric esters, and another stabilizing and gelatinizing compound also possessing both these properties one of the two gelatinizing and stabilizing compounds possessing 75 the first mentioned property to a smaller extent and the second mentioned property to a larger extent than the other gelatinizing and stabilizing compound.

In testimony whereof we have signed our 80 names to this specification in the presence of subscribing witnesses.

FREDERIC LEWIS NATHAN.  
WILLIAM RINTOUL.

Witnesses:

M. B. MITRIE,  
ALEX FORBES.

HENRY BAKER,  
*Administrator of the estate of Frank Baker, deceased.*

Witnesses:

BERTRAM H. MATTHEWS,  
P. A. OUTHWAITE.